

# UNITED STATES PATENT OFFICE.

CHARLES M. DABOLL, OF NEW LONDON, CONNECTICUT.

## HARDENING METALS.

SPECIFICATION forming part of Letters Patent No. 255,725, dated March 28, 1882.

Application filed August 25, 1881. (No specimens.)

To all whom it may concern:

Be it known that I, CHARLES M. DABOLL, of New London, in the county of New London and State of Connecticut, have invented certain new and useful Improvements Relating to Hardening Metals, of which the following is a specification.

I have experimented on what are known as "roller-bushings" in the sheaves of pulley-blocks for use on shipboard and in other situations. The usefulness of these bushings depends largely upon the maintaining of the sizes and proportions of the members of the complex structure. Economy requires that the whole be made cheaply. I make all the parts of common cast-iron, cast in sand in the ordinary manner, with the smallest cost and with the moderate hardness due to ordinary castings thus made. I finish the parts while in the ordinary soft condition. Then, without any long process and without requiring expensive labor, I harden the finished castings without distorting or warping them. The surface produced by the treatment is a good protection against oxidizing influences.

My hardening is effected more quickly and cheaply than case-hardening, and the hardness is different. The castings are hardened quite through. It will of course be understood that the posts which traverse the spaces between the rings and hold them together are made of metal which will rivet. The other parts—rollers, shell, rings, and, if desired, the entire sheave—may be cast-iron, accurately finished and hardened. I believe that for all the purposes for which chain and rope sheaves are required the parts will maintain their exact size and condition indefinitely.

All the parts are cast of ordinary iron, and then reduced to the exact size and form by tools acting on it in a soft condition.

I employ a hardening-trough containing a solution compounded as follows: Forty gallons of pure water, fifty pounds of common rock-salt, two pounds of saltpeter, two pounds of cyanide of potassium, five pounds of the ordinary sulphuric acid of commerce. The solution should be kept cold or at as low a temperature as the active use in cooling large numbers of small castings will allow.

Care should be taken to heat the parts sepa-

rately or to so support them as not to distort the forms or bruise or in any wise injure the surfaces which require to work together. They should be plunged into the solution endwise. 55

Castings one and one-half (1½) inch through have by my treatment been hardened entirely through, and I believe much larger ones can be similarly hardened quite evenly through with proper apparatus to move each rapidly 60 to a considerable depth at the instant of immersion. The nature of the metal is materially changed by the process. They should be allowed to lie in the solution a few minutes after the cooling. The hardening is completed at the 65 moment of cooling, but the solution affects the surface more thoroughly by being allowed to remain. It contributes to give more perfectly the fine blue-black oxide, which is one result of my operation. On removal from the harden- 70 ing-bath they are soaked a considerable time in water containing lime to neutralize any acid remaining in the pores. They are then dried, applied together, inserted in the sheave, and introduced in the block. 75

The pin, which is fixed in the block and serves as a fixed axis, is of my hardened cast-iron, similarly made and hardened.

It is important that all the elements be employed, but the proportions may be varied 80 within considerable limits. I esteem the cyanide of potassium especially important. The proportion thereof should not be much less than above indicated. The cost of the whole is insignificant. Little time is consumed. No 85 expensive furnaces or boxes or packing are required. The whole may be operated with the ordinary tools and appliances of a small foundry and machine-shop.

The body of the sheave may be of any material—composition, cast-iron, galvanized, or lignum-vitae or other hard wood.

The shell may have a flange and fastening-rivets. The hardened bushing may be inserted in the metallic sheave by driving, pressing, 95 pinning, or any other ordinary or suitable way. When the body of the sheave is of iron the shell may be dispensed with and the body of the sheave itself cast in the proper form, and milled or turned out to receive the rollers directly. In such case the entire sheave should be hardened in my solution. It will be under-

stood that the block may be wood or metal, and widely varied as to form, number of sheaves, mode of strapping, &c.

5 The pin may be cylindrical steel, hard iron, or any other ordinary material.

The articles herein described as hardened will be made the subject of a separate application for patent.

I claim as my invention—

10 The hardening solution described, composed of water, sulphuric acid, salt, saltpeter, and

cyanide of potassium, combined in about the proportions herein specified.

In testimony whereof I have hereunto set my hand, at New London, Connecticut, this 15 20th day of August, 1881, in the presence of two subscribing witnesses.

CHARLES M. DABOLL.

Witnesses:

CHARLES ALLISON,  
A. H. AVERY.